

## UNITED STATES PATENT OFFICE

2,442,120

MAKING OF BARITE CONCENTRATES  
USEFUL IN DRILLING MUDS

James B. Duke, Lakeland, Fla., assignor to Minerals Separation North American Corporation, New York, N. Y., a corporation of Maryland

No Drawing. Application May 12, 1945,  
Serial No. 593,530

4 Claims. (Cl. 23—122)

1

This invention relates to the making of barite concentrates useful in drilling muds.

Barite concentrates which have been produced by froth-flotation, agglomeration table concentration or other methods involving the use of anionic reagents, are largely non-wettable because of the residues of reagents left on the barite particles. In this non-wettable state, such barite concentrates are not satisfactory for use in the making of drilling muds used in the petroleum oil industry because, in the making of the muds, much air is entrained thereby lowering the specific gravity of the muds.

In order to make such concentrates wettable, it has been customary to subject them to drying and calcining heat treatments which destroy the reagents on the barite particles. The calcining heat treatment is expensive and difficult to control, since if the temperature to which the concentrates are subjected is too low the reagents on the barite particles are not destroyed, and if the temperature is too high some of the barite is converted into black ash (barium sulphide). By treating the barite concentrates in accordance with the present invention, this expensive and troublesome calcining heat treatment is eliminated.

The reagents left on the barite particles after froth-flotation concentration are the cause also of other difficulties. For example, these concentrates must be dewatered before drying, and the reagents left on them tend to interfere with proper settling of the concentrates in such dewatering equipment as thickeners, cones, rake classifiers etc., with resulting large overflow losses and high circulating loads which are a source of never-ending trouble in plant operations.

The present invention is the result of the discovery that treatment of barite concentrates (produced by froth-flotation, agglomeration table concentration or other methods involving the use of anionic reagents in an aqueous pulp of the ore) with a strong mineral acid, followed by the washing of the acid-treated concentrates substantially free of acid and slimes, results in such substantially complete removal of the reagents from the barite particles that the operations in thickener tanks, mechanical cones and rake classifiers are substantially free of the difficulties hereinbefore mentioned; and the further discovery that the acid-treated and washed barite concentrates, after being dried and ground to the

necessary fineness (usually about —325 mesh) are in a completely wettable state and suitable for use in the making of drilling muds. The economies in plant operation achieved by the invention are important, and the quality of the final barite product is improved.

The invention will be understood from the following description of several examples showing how the wettability of barite flotation concentrates is increased by the use of the invention. In Examples I to IV, the barite concentrates were produced in the usual way by froth-flotation treatment of a barite ore which had been ground to about minus 35 mesh, and subjected to substantial desliming which resulted in getting rid of most of the minus 150 mesh material. The flotation agents employed in these examples were of the usual kind, namely, caustic soda, fuel oil, and red oil (oleic acid) or a material known as "Varlacoid" which is a mixture of fatty and resin acids. In Examples V and VI, the barite concentrates which were treated in accordance with the invention were produced by froth-flotation operations in a commercial barite concentrating plant. The strong mineral acids used in Examples II, IV, V and VI which illustrate the practice of the invention, were sulfuric acid, nitric acid and hydrochloric acid, and from the success achieved by the use of these acids the conclusion is justified that strong mineral acids generally are satisfactory in practicing the invention.

*Example I.—Without acid treatment*

The barite ore after being ground and substantially deslimed, as above mentioned, was conditioned in an aqueous pulp at about 72% solids for two minutes with 0.2 lb. caustic soda, 4.7 lbs. fuel oil and 1.0 lb. red oil (oleic acid), all per ton of solids in the feed. The thus conditioned barite ore pulp was then subjected to froth-flotation treatment with the following metallurgical results:

| 45    | Products | Per Cent Wt. | Per Cent BaSO <sub>4</sub> | BaSO <sub>4</sub> Per Cent Distribution |
|-------|----------|--------------|----------------------------|-----------------------------------------|
| Feed  |          | 100.0        | 69.2                       | 100.0                                   |
| Cone  |          | 70.4         | 93.5                       | 95.1                                    |
| Mid-3 |          | 1.3          | 74.4                       | 1.4                                     |
| Mid-2 |          | 1.5          | 61.3                       | 1.3                                     |
| Mid-1 |          | 2.3          | 32.2                       | 1.0                                     |
| Tail  |          | 24.5         | 3.3                        | 1.2                                     |

The barite concentrates thus obtained were de-watered and air-dried overnight. When a portion of these barite concentrates was submerged in water, large flocs or agglomerates were formed immediately when the particles came in contact with the water, and it was impossible to wet these agglomerates by stirring. Another portion of the air-dried concentrates was then ground to minus 325 mesh, and when this finely ground portion was submerged in water the major portion of it still formed large agglomerates which it was impossible to wet by stirring. This example illustrates the non-wettability of barite concentrates produced by the usual froth-flotation methods involving the use of reagents in an aqueous pulp of the ore.

*Example II.—With sulfuric acid treatment*

In this example, the barite ore was the same as in Example I and the flotation reagents were the same; but the final flotation concentrates were agitated at approximately 50% solids for about three minutes in an aqueous pulp containing 5.0 lbs. sulfuric acid per ton of solids; after which the acid-treated barite concentrates were washed substantially free of acid and slimes. The thus treated concentrates were then de-watered and air-dried overnight. When a portion of these dried concentrates was submerged in water, approximately 30% of the concentrates were not wetted by the water and formed agglomerates. When, however, another portion of these same air-dried concentrates was ground to approximately minus 325 mesh and was submerged in water, approximately 99% of the concentrates appeared to be wetted by the water, and no visible agglomerates were formed. This proves that acid-treatment of the barite flotation concentrates, followed by washing and fine grinding, produces barite concentrates which are satisfactory for use in the making of drilling muds.

*Example III.—Without acid treatment*

In this example, the barite ore and the treatments thereof were the same as in Example I, except that 1.0 lb. of Varlacoid, per ton of solids in the ore, was substituted for the red oil. As before, the acid-treated and washed flotation concentrates were air-dried overnight. When a portion of these air-dried concentrates was submerged in water, approximately 50% of the material was not wetted by the water and formed large agglomerates which it was impossible to wet by stirring. Also, when another portion of the air-dried concentrates was ground to minus 325 mesh and submerged in water, substantially all of the material appeared to form very small flocs with some of the material as a froth on the surface of the water. As in the case of Example I, this example illustrates the non-wettability of barite flotation concentrates which have not been subjected to treatment to make them wettable.

*Example IV.—With sulfuric acid treatment*

In this example, the barite ore was the same as in Example III, and the barite flotation concentrates were produced with the same flotation agents. These barite flotation concentrates were agitated in an aqueous pulp at approximately 50% solids with 5.0 lbs. of sulfuric acid, per ton of solids, for about 3 minutes; after which the concentrates were washed substantially free

of acid and slimes, were de-watered and air-dried overnight. When a portion of these air-dried concentrates was submerged in water, approximately 98% of the material appeared to be wetted by the water; and, when another portion was ground to minus 325 mesh and submerged in water, all of the material appeared to be wetted by the water. Therefore, this example, like Example II, proves that acid treatment of barite flotation concentrates followed by washing, drying and fine grinding, produces a material which is satisfactory for use in the making of drilling muds.

*Example V.—With nitric acid treatment*

The purpose of this example is to show that nitric acid, instead of sulfuric acid, may be employed in practicing the invention. The barite flotation concentrates were obtained from a commercial plant engaged in concentrating barite by froth-flotation treatments with the usual reagents. A portion of these barite concentrates was agitated in an aqueous pulp for about three minutes with 14 lbs. of nitric acid per ton of solids; after which the acid-treated concentrates were washed with water until the acid and slimes were substantially removed. The acid-treated and washed concentrates were then de-watered and dried by heat treatment at a fairly low temperature, care being taken not to burn the concentrates. After the thus dried barite concentrates had cooled, a portion of them was submerged in water; with the result that although approximately 70% of the material was easily wetted, the other 30% was found to be very difficult or impossible to wet. When, however, another portion of the dried barite concentrates was ground to minus 325 mesh and submerged in water, all of it was easily wetted. Thus, this example proves that nitric acid may be satisfactorily used in practicing the invention.

*Example VI.—With hydrochloric acid treatment*

In this example, as in Example V, the barite concentrates subjected to treatment according to the invention were obtained from a commercial plant engaged in concentrating barite by the usual froth-flotation methods. In this case, the barite concentrates were agitated in an aqueous pulp with hydrochloric acid in the amount of 14 lbs. per ton of solids in the pulp, and were then washed substantially free of acid and slimes. This produced barite concentrates which, after drying and fine grinding, were readily wettable and as satisfactory for use in drilling muds as in the cases of the barite concentrates which were treated with sulfuric acid or nitric acid as described in Examples II, IV and V.

What is claimed is:

1. The method of treating barite concentrates which are coated with reagents owing to having been produced by flotation or agglomeration methods involving the use of anionic reagents in an aqueous pulp of the barite ore, to make said barite concentrates wettable and useful in drilling muds, which comprises agitating said concentrates in an aqueous pulp containing a strong mineral acid selected from the group consisting of sulfuric, nitric and hydrochloric acids, washing said acid-treated pulp substantially free of acid and slimes, drying the thus treated barite concentrates, and grinding said dried concentrates to the fineness required in drilling muds.

2. The method according to claim 1 in which the mineral acid is sulfuric acid.  
 3. The method according to claim 1 in which the mineral acid is nitric acid.  
 4. The method according to claim 1 in which the mineral acid is hydrochloric acid.

JAMES B. DUKE.

## REFERENCES CITED

The following references are of record in the file of this patent:

## UNITED STATES PATENTS

| Number    | Name                 | Date          |
|-----------|----------------------|---------------|
| 1,102,873 | Chapman et al. ----- | July 7, 1914  |
| 1,365,281 | Scott -----          | Jan. 11, 1921 |
| 1,575,945 | Straud -----         | Mar. 9, 1926  |
| 2,371,292 | Hoag -----           | Mar. 13, 1945 |

## OTHER REFERENCES

10 Clemmer et al., U. S. Bureau of Mines Report of Investigations No. 3239, pages 14 and 15. "Title: Flotation and depression of nonsulphides: calcite, silica and silicates, fluorspar, barite, apatite, and tungsten minerals.